

Patented Aug. 23, 1927.

## UNITED STATES PATENT OFFICE.

OLIVER W. STOREY AND GORDON T. COLLINSON, OF MADISON, WISCONSIN, ASSIGNEES  
TO C. F. BURGESS LABORATORIES, INC., OF DOVER, DELAWARE, A CORPORATION  
OF DELAWARE.

PRODUCING OXIDIZED CARBON.

No Drawing.

Application filed July 7, 1925. Serial No. 42,111.

This invention relates to the electrochemical production of solid carbon oxide or oxides having the properties of graphitic oxide.

5 In a copending application of Bruce K. Brown, Serial No. 42,091, filed July 7, 1925, a method for the electrochemical production of carbon oxides is disclosed. This method consists in mounting carbonaceous material 10 as anode in an oxidizing electrolyte, such as 30% nitric acid at about room temperature, and passing an electric current having a density of about ten amperes per square foot of anode surface. The anode disintegrates to a sludge which is a mixture of 15 carbon and oxide of carbon and may contain as high as 6% by weight of available oxygen. Carbon so oxidized does not have the yellow color of pure graphitic oxide but 20 has the dull black appearance of partially oxidized carbon and it apparently is identical or approximately identical with the product obtained by chemical oxidation. We have found that the yield and oxygen percentage of the oxidized carbon product may 25 be greatly increased by suitably treating the electrodes that are to be disintegrated and further by the maintaining of the cell at the proper temperature while using electrodes so treated.

30 If a graphitic or other carbonaceous electrode is used as an anode in a dilute nitric acid or other suitable electrolyte for the production of oxidized carbon, the electrode 35 disintegrates at a rate depending upon the composition of the electrolyte, current density, temperature of the electrolyte, and composition of the electrode. Usually, an untreated anode which is disintegrated in dilute 40 nitric acid at room temperature disintegrates into a product that varies over a wide range of particle sizes. The coarser particles may be as large as walnuts while the finer particles may pass through a 100 mesh screen.

45 All of these particles have a coating of 45 oxidized carbon. It is readily seen that on a weight basis the coarser particles have a relatively small percentage of fixed oxygen whereas the small particles will have a high percentage if the coating is of the same

thickness on all particles. This is borne out in practice, since the finely disintegrated product is found to have the higher percentage of available oxygen. As an illustration, if that part of the product from 55 an untreated graphite anode which will pass through 100 mesh has an available oxygen percentage of about 5 percent, that part of the product which passes through 40 mesh but is retained on 100 mesh will have an 60 available oxygen percentage of about 4 percent. Similarly the percentage of oxygen gradually decreases as the particles increase in size, until the coarsest particles contain considerably less than 1 per cent of oxygen. 65 While it is possible to utilize such a product industrially by screening out the coarser lumps, the coarse lumps represent a considerable loss, as they often constitute 25 per 70 cent or more of the entire product.

We have found that the physical disintegration of the anodes results from the penetration of the electrolyte into the pores of the electrode. The ordinary molded electrode is porous to a considerable degree and 75 in the case of graphite even the individual particles are porous to the extent that they are laminated. As the electrolyte penetrates into the pores of the electrode, the current finds a path into the interior of the electrode. The electrolysis of the oxidizing electrolyte in the pores of the carbonaceous material results in the oxidation of the carbon to a solid oxide of carbon. The formation 80 of the solid oxide is accompanied by a perceptible increase in volume or swelling. This causes physical disintegration. We have found that this may be stopped. The remedy is to prevent the electrolyte from entering 85 the pores of the electrode.

The easiest method of preventing the electrolyte from entering the pores of the electrode is to fill these pores with a water repellent, such as paraffin. Paraffining the electrode is easily carried out and it is very 95 effective in preventing the formation of large lumps, in fact, a product can be made all of which will pass through a 20 mesh screen and 95 per cent of which will pass 100 through a 60 mesh screen.

Not only does the paraffin prevent the disintegration of the electrode into large lumps but it also raises the percentage of fixed oxygen. If an untreated graphite electrode is 5 disintegrated in a dilute nitric acid electrolyte, the fixed oxygen in the product passing through a 60 mesh screen will be approximately five percent. By paraffining the anode, the disintegration product passing 10 through 60 mesh will contain between 9 and 10 percent of oxygen. The increase in the fixed oxygen content obtained when an electrode is saturated with paraffin can probably be explained on the theory that 15 the electrolyte is prevented from penetrating the pores of the carbon, and instead, allows the electrolyte to penetrate the particles of carbon and thereby rupture these. In the case of graphite, the electrolyte no 20 doubt penetrates between the laminations, whereas this probably does not occur when the graphite is unparaffined. The paraffining results in a much better penetration of the individual particles in contrast to the 25 penetration of the electrolyte into the spaces around the separate particles when unparaffined. The paraffining of an anode may be carried out by immersing it in smoking-hot melted paraffin for a time long enough to 30 effect complete penetration.

While paraffining of the electrode is a cheap and efficient method for securing a disintegration into fine particles by confining this disintegration and oxidation to the 35 surface of the electrode in contact with the electrolyte, it is possible to use a wide variety of similar wax-like and other water repellent materials such as rosin. It is also possible to use ordinary lubricating oils. 40 Discarded crank case oil is a cheap and efficient oil which may be used to displace the more expensive refined oils. The electrodes may even be saturated with gasoline, naphtha, carbon tetrachloride and similar solvents, preferably those not easily attacked 45 by the oxidizing reactions at the anode. Their effect, however, is not as permanent, since they are gradually driven out during the electrolysis, so that the product contains 50 particles of increasing size as the electrolysis proceeds.

It is not necessary to use oils, waxes, or solvents of a water repellent nature, as any 55 material will work which will prevent diffusion of the electrolyte and confine the oxidation and disintegration to the surface of the electrode in contact with the electrolyte. An electrode thoroughly soaked in water will show the characteristics of a paraffined anode for a time until the electrolyte has so diffused into the interior that the liquid in the pores becomes conductive enough 60 to conduct the current sufficiently to cause electrochemical oxidation. The electrode 65 may be saturated with water solutions of

various chemical reagents which will cut down the rate of electrolyte diffusion.

It is also possible to saturate the electrode with a solution of a reagent such as sodium silicate which will form an insoluble precipitate or gel when it comes in contact with the electrolyte and will thereby prevent diffusion into the interior of the electrode. The precipitate should be of such a nature that it may be subsequently washed out of the 70 oxidized carbon, or if it is not washed out, should be harmless for the uses to which the oxidized carbon is put.

After the disintegration of the electrode, the powdered material is washed with water 80 to remove the electrolyte or other chemicals that may be present. If a moisture repellent is used to saturate the electrode, this material is found in the disintegration product. This may be removed by suitable solvents, especially such solvents as boil below 100° C. If the oxide of carbon has to be heated much above 100° C. there is an appreciable deterioration of the oxide. Carbon tetrachloride is an efficient extracting 90 agent when paraffin is used for saturating the electrode. It has the distinct advantage of not being flammable but has the disadvantage of high cost. Benzole is also an effective agent, while ordinary gasoline has 95 high boiling fractions present which cannot be driven readily from the colloidal oxide of carbon. The moisture repellent may be extracted in the cold but is more easily removed by boiling under a reflux condenser 100 and washing with pure solvent, though this procedure tends to drive off some of the oxygen also. The solvent and the moisture repellent may be recovered by distillation. If carbon tetrachloride or similar volatile 105 solvents are used for saturating the electrodes during electrolysis it does not become necessary to extract these from the oxide of carbon. Simply heating the oxide to above the boiling point of the solvent drives 110 off the solvent. The advantages of this procedure are apparent.

If the oxide of carbon is used for depolarizing purposes in electric batteries it is essential that practically all of the moisture 115 repellent be extracted. Even small amounts of paraffin will greatly decrease the conductivity of the material. Great difficulty is also experienced in wetting the materials when made up into a depolarizing mixture 120 for dry cells.

The temperature of the electrolyte is an important factor for the securing of high yields and high percentages of fixed oxygen. As in the case of untreated electrodes, when 125 the temperature is elevated, the yield decreases. With paraffined electrodes, the best conditions seem to be at room temperature, approximately 20° to 25° C. When benzole is used as the impregnating agent, the best 130

results are obtained below 0° C. At this low temperature the benzole freezes and acts as a solid moisture repellent. At ordinary temperatures the benzole is apparently oxidized more rapidly than the carbon and in some of our experiments has decreased the yield of oxidized carbon. These results indicate that it is preferable to have a saturating medium which will be less readily oxidized than the carbon, or the temperature should be so regulated that this condition is realized, as in the case of the benzole.

Throughout the specification and claims carbon is used in the broader sense and includes the graphitic state of the element. Carbonaceous material is used throughout the specification and claims to cover a material containing free carbon in any of its allotropic forms.

20 We claim:

1. The method of producing pulverous, oxidized carbon consisting essentially of submitting an anode of carbon which has been treated to confine the oxidation and disintegration of the electrode to the surface in contact with the electrolyte to an electric current in a bath having an oxidizing oxygen containing anion.

2. The method of producing pulverous, oxidized carbon all of which will pass through a 20 mesh screen consisting essentially of submitting an anode of carbon which has been treated to confine the oxidation and disintegration of the electrode to the surface in contact with the electrolyte to an electric current in a bath having an oxidizing oxygen containing anion.

3. The method of producing pulverous, oxidized carbon consisting essentially of submitting an anode of carbon that has been impregnated with a moisture repellent to an electric current in a bath having an oxidizing oxygen containing anion.

4. The method of producing pulverous, oxidized carbon all of which will pass through a 20 mesh screen consisting essentially of submitting an anode of carbon that has been impregnated with a moisture repellent to an electric current in a bath having an oxidizing oxygen containing anion.

5. The method of producing pulverous, oxidized carbon consisting essentially of submitting an anode of carbonaceous material that has been impregnated with a moisture repellent which is solid at atmospheric temperatures to an electric current in a bath having an oxidizing oxygen containing anion.

6. The method of producing pulverous, oxidized carbon consisting essentially of submitting an anode of carbonaceous material impregnated with a moisture repellent more resistant to the electrolyte and to the oxidizing reaction at the anode than the car-

bonaceous material of such anode to an electric current in a bath having an oxidizing oxygen containing anion.

7. The method of producing oxidized carbon in pulverous form consisting essentially of submitting an anode of carbonaceous material that has been impregnated with paraffin to an electric current in a bath having an oxidizing oxygen containing anion.

8. The method of producing pulverous, oxidized carbon consisting essentially of submitting an anode of carbon that has been impregnated with a moisture repellent to an electric current in a bath having an oxidizing oxygen containing anion and leaching with water the product so formed.

9. The method of producing pulverous, oxidized carbon consisting essentially of submitting an anode of carbon that has been impregnated with a moisture repellent to an electric current in a bath having an oxidizing oxygen containing anion and leaching the product so formed with water and with a solvent capable of extracting the moisture repellent.

10. The method of producing pulverous, oxidized carbon consisting essentially of submitting an anode of carbon that has been impregnated with a moisture repellent to an electric current in a bath having an oxidizing oxygen containing anion and leaching the product so formed with water and benzol.

11. The method of producing pulverous, oxidized carbon consisting essentially of submitting an anode of carbonaceous material that has been impregnated with a moisture repellent to an electric current in a bath containing nitric acid.

12. The method of producing pulverous, oxidized carbon consisting essentially of submitting an anode of carbonaceous material that has been impregnated with a moisture repellent to an electric current in a bath containing nitric acid and sodium dichromate.

13. The method of producing oxidized carbon consisting essentially of submitting an anode of carbonaceous material that has been impregnated with paraffin to an electric current in a bath having an oxidizing oxygen containing anion and leaching the product so formed with water and benzol.

14. The method of producing oxidized carbon consisting essentially of submitting an anode of carbonaceous material impregnated with a moisture repellent to an electric current in a bath having an oxidizing oxygen containing anion at a temperature below 50° C.

15. The method of producing oxidized carbon consisting essentially of submitting an anode of carbonaceous material impregnated with a moisture repellent to an electric current in a bath having an oxidizing oxygen containing anion at a temperature of approximately 20° C.

16. The herein described product consisting essentially of a mixture of carbon and oxidized carbon in pulverous form capable of passing through a 20 mesh screen and containing a moisture repellent.

17. The herein described product consisting essentially of oxidized carbon in pulver-

ous form capable of passing through a 20 mesh screen and containing a moisture repellent.

10 In testimony whereof we affix our signatures.

OLIVER W. STOREY.  
GORDON T. COLLINSON.